

Patented Aug. 7, 1945

Tx 106/15.05

X

2

## UNITED STATES PATENT OFFICE

2,381,852

## TREATMENT OF TEXTILES

Carroll A. Hochwalt, Montgomery County, Ohio,  
assignor to Monsanto Chemical Company, a  
corporation of Delaware

No Drawing. Application March 16, 1942,  
Serial No. 434,832

6 Claims. (Cl. 117—138.5)

This invention relates to a process for the treatment of fibrous materials and more specifically to a process whereby textiles are simultaneously protected from attack by fungi and bacteria and rendered moisture-proof.

Much damage is caused to fibrous materials by fungi and bacteria. Mildew, that is, the growth of fungi on fibrous media, is characterized by discoloration of the media and the development of a musty smell accompanied by decay or rotting of the fiber. This is caused by utilization of certain constituents of the fiber in the metabolic processes of fungi and bacteria, and is usually characterized by loss of strength of the fiber. Since the main factors determining micro-biological growth are food and moisture, and since the cellulose of cotton, hemp, jute, etc., and the protein, fat and gum constituents of wool and silk provide ready food for fungi and bacteria these fibers and textile materials made therefrom may be readily attacked by such micro-organisms under proper moisture conditions. Storage of fibrous materials in damp warehouses, exposure to rain without immediate drying, as in the case of tents, tarpaulins, awnings, etc., and use of fibrous materials, for example, fish nets, under conditions of constant wetting provide favorable moisture conditions for the growth of fiber-destroying fungi and bacteria.

The problem of protecting fibrous materials against the attack of these microorganisms has been complicated by certain stringent requirements. The mere gross surface application of substances possessing fungicidal and bactericidal properties is often inadequate in that it does not prevent attack by microorganisms which may have been previously deposited within the fiber. The impregnation of fibrous materials with fungicides and bactericides often results in the impairment of the strength of the fibrous material by the impregnating agent. Again, an otherwise satisfactory impregnating agent may be unsuitable for many purposes in that it may be readily leached out of the treated material by rain, by washing, etc.

The following properties may be considered as being desirable in a fungicidal and bactericidal material for the treatment of textiles: (1) It must possess both fungicidal and bactericidal properties. (2) It should be neither acid nor

alkaline. (3) It must be insoluble or only slightly soluble in water to avoid leaching out by rain. (4) It should not increase inflammability. (5) It should not detract from fiber strength. (6) It must be readily available and easily applied. (7) It should not cause excessive shrinkage. (8) It should not unfavorably affect the feel of the material treated.

An object of the present invention is the provision of new textile treating processes and products whereby there are used fungicidal and bactericidal materials having particularly desirable qualities. Another object of the present invention is the provision of a process whereby textiles are simultaneously protected from attack by fungi and bacteria and at the same time rendered moisture-proof and water repellent. Other objects and advantages will hereinafter become apparent.

10 By the process of the present invention a fibrous material, for example, cotton cloth, may first be treated with an aliphatic dibasic acid or anhydride or salt thereof having as a substituent an olefinic hydrocarbon residue of from 5 to 16 carbon atoms and then with a water soluble copper salt. The alkylene, e. g., amylene, hexylene, heptylene, octylene, diisobutylene, triisobutylene or tetraisobutylene, substituted dibasic acids or anhydrides used may be prepared by reaction 15 of a salt of an unsaturated dibasic acid or by reaction of the anhydride with an aliphatic hydrocarbon having an olefinic double bond as described in U. S. Patent 2,055,456 to Eichwald. Such alkylene substituted acids or anhydrides are 20 relatively insoluble in water and for the purpose of expediting their application to the cellulosic material I may convert them by known methods to their water-soluble alkali metal salts whereby I operate by first treating the cellulosic material 25 with the aqueous solution of the alkali metal salt of the alkylene dibasic acid then with a solution of the soluble copper salt. If desired, however, I may treat the fibrous material by a one-step process wherein I first prepare the relatively 30 water-insoluble copper salt of the alkylene dibasic acid and apply it to the cellulosic material, for example, in the form of an aqueous dispersion prepared with the aid of a dispersing agent.

35 Thus my invention includes the production of 40 copper salts (cupric or cuprous) of alkylene

45

50

succinic acids, such salts having the probable constitution:



where R is an alkylene residue of from 5 to 16 carbon atoms.

In practice I may operate as follows: I treat a textile material, for example, cotton cloth, in a padding machine at room temperature for from 5 to 10 minutes in, say, a 1% to 20% aqueous solution of an alkali metal salt of triisobutylene succinic acid, dry the cloth at approximately 90° C. in a draft oven, and then treat it in a padding machine with, say, a 1% to 5% aqueous solution of cupric acetate. After a short rinse I air-dry the cloth and may then bake it for from 10 to 60 minutes at 120 to 160° C.

The effect of the treatment of fabrics by the present process upon change in tensile strength, may be determined by the method described in the American Society for Testing Materials Book of Standards for 1939, part III on pages 364 and 372. Breaking strengths as determined by means of a Model J-2 Scott Tester, using American Society for Testing Materials Specification D39-36 raveled strip method, as described on these pages, indicate that cloths treated according to the process of this invention undergo substantially no change in tensile strength.

Fabrics treated according to the process may also be evaluated as to fungus resistance by inoculating them with a culture of *Chaetomium globosum*, one of the most destructive of the fiber-attacking fungi, and allowing the so inoculated fabric to stand for two weeks under favorable conditions for growth. Since attack by the fungus results in loss of tensile strength, the effect of the inoculated *Chaetomium globosum* upon the fabric may be readily estimated by measuring the tensile strength of the fabric before inoculation and after the two-week exposure. Cloths treated according to the process of this invention show substantially no loss of tensile strength after inoculation and exposure to the fungus as above described.

The water repellency of the fabrics treated by the herein described process may be evaluated by two tests applied by those skilled in the art. These tests are known as the "spray test" and as the "hydrostatic head test." The spray test which I employ is described in the American Dyestuffs Reporter, vol. 28, page 285 for 1939. The hydrostatic head test is described in the 1940 Yearbook of the American Association of Textile Chemists and Colorists at pages 223-4. Fabrics treated by the process of this invention show percentage absorption values and hydrostatic head values which indicate good water-resistance.

The herein described process is especially valuable for the simultaneous rot-proofing and moisture-proofing of the various textile fibers or fibrous products, namely fabrics woven from cotton, linen, wool, jute, artificial silk, yarns and the like. The process may also be applied to paper forming fibers such as sulfate, sulfite and ground wood pulp, or to paper, itself.

This invention is illustrated but not limited by the following examples:

### Example 1

A 6" by 50" piece of Indian Head cloth is run at room temperature for 8 minutes through a padder in approximately 500 cc. of a 1% benzene solution of triisobutylene succinic anhydride and the treated cloth is then air-dried and baked for one hour at 150° C. At the end of this time the cloth is padded with a 1% aqueous solution of cupric acetate, rinsed to remove unreacted copper acetate, allowed to dry in the air, and then baked for one hour at 150° C. The treated cloth will be found to have permanent, water-resistant fungicidal and bactericidal properties, water-repellency and good feel. Its inflammability will not have been increased, and its tensile strength will not have been impaired by the treatment.

The cloth was found to have a tensile strength of 43.3 pounds as measured on the Scott tester, before inoculation and a tensile strength of 43.6 pounds after inoculation and exposure for two weeks under conditions favoring growth of the fungus. Thus the cloth suffered no loss of strength due to exposure to moisture and fungicidal action.

The treated cloth showed the following degree of water-proofness: Tested with the spray test above referred to, I obtained a moisture absorption of 32.1% and a hydrostatic head value of 21.2 cm., which values indicate good water-resistance.

### Example 2

The procedure is that of Example 1, except that instead of using a 1% solution, there is used a 5% solution of triisobutylene succinic anhydride in benzene. When the treated cloth was evaluated for fungicidal property as described herein, the tensile strength of the cloth after exposure to the fungus was found to be 44.0 pounds as against 43.1 pounds, the value obtained for the cloth before inoculation.

The treated cloth of this example showed the following degree of water-proofness. Tested with the spray test and the hydrostatic head test above referred to, I obtained a moisture absorption of 28.2% and a hydrostatic head value of 21.2 cm.

Instead of the triisobutylene succinic anhydride of the above examples I may use the triisobutylene succinic acid, itself. Moreover when operating in a non-aqueous media I may use benzene as the solvent or I may use any other inert diluent, as will be understood by those skilled in the art. If it is desired to operate in an aqueous media, I may prepare, say, the disodium salt of triisobutylene succinic acid and apply it to the cellulosic material in the form of, say, a 2% to 20% aqueous solution. Textiles treated with such aqueous solutions of disodium triisobutylene succinate when submitted to subsequent treatment with a 1% to 5% aqueous solution of cupric acetate show the incorporation therein of from 0.35% to 1.3% copper, based on the weight of the dry textile.

Although the above examples illustrate the operation of this invention by a two-step process, the formation of the copper salt of triisobutylene succinic acid being advantageously precipitated directly upon the fiber, I may likewise operate by a one-step process, by first preparing the copper salt, for example by reaction of the triisobutylene succinic acid with cupric or cuprous acetate, and then applying it to the textile material. Cupric triisobutylene succinate, for example, may be

15

2,381,852

3

applied to the cellulosic material by preparing an aqueous dispersion of the salt. While such a dispersion can be prepared mechanically, its preparation is somewhat easier if the cupric triisobutylene succinate is dispersed in the presence of dispersing agents such as copolymers of styrene and maleic anhydride, which copolymers have been converted to their water-soluble salts.

Instead of using triisobutylene succinic acid or its salts for the purpose of the present invention, I may likewise use the alkylene substituted succinic acids or their salts prepared by reaction of such olefinic hydrocarbons as amylene, hexylene, octene, dodecene, etc., with maleic acid or maleic anhydride, the use of such alkylene succinic acids according to the present invention likewise resulting in rendering fungicidal, bactericidal and moisture-proof properties to cellulosic materials. Although I prefer to employ the products obtained from maleic acid or its anhydride because these compounds are readily available on a commercial scale, I may likewise use the other alkylene derivatives of aliphatic dibasic acids described in U. S. Patent 2,055,456, for example the products obtained by reaction of olefinic hydrocarbons containing from 5 to 16 carbon atoms with such acids as fumaric acid, citraconic acid or itaconic acid.

What I claim is:

1. The compound having the formula:



where R is an alkylene residue of from 5 to 16 carbon atoms.

2. A textile fiber, the surfaces of which contain the cupric salt of an acid of the formula:



10 where R is an alkylene residue of from 5 to 16 carbon atoms.

3. The process of treating textile fibers to render the same water-repellent and resistant to rot development, comprising treating said fibers with a monoalkylene succinic acid salt, the alkylene group of which contains from 5 to 16 carbon atoms and thereafter treating said fibers with a soluble cupric salt.

15 4. The process defined in claim 3 in which the soluble copper salt is cupric acetate.

5. The process of treating textile fiber to render the same water repellent and also resistant to the development of fungus organisms of the character of *Chaetomium globosum*, which comprises treating said fiber with an aqueous solution of the disodium salt of triisobutylene succinic acid, thereupon treating said fibers with a solution of a soluble copper salt and then drying said fibers.

20 6. A fibrous textile product, the fibers of which carry sufficient of the cupric salt of triisobutylene succinic acid, so that said product in the dry state contains from 0.35% to 1.3% of copper.

25 35 CARROLL A. HOCHWALT.